

## UNITED STATES PATENT OFFICE

2,396,670

## PROCESS FOR MODIFYING FATTY OILS

Laszlo Auer, South Orange, N. J.

No Drawing. Application October 12, 1942,  
Serial No. 461,789

23 Claims. (Cl. 106—222)

GENERAL FIELD OF INVENTION AND STATEMENT OF  
OBJECTS

This invention relates to the modification of fatty oils. The present application is a continuation-in-part of my copending application Serial No. 383,339 filed March 14, 1941, now Patent No. 2,298,915 issued October 13, 1942.

Fatty oils are employed in a number of different industries, such, for instance, as the coatings and plastics industries, and it is a general object of this invention to modify and improve the properties of fatty oils for various industrial purposes.

Briefly, the invention contemplates treatment of a fatty oil, for instance linseed oil, with fluorescein, with application of heat. Full description of the treatment procedure is given hereinafter.

According to the present invention it is possible to achieve a number of advantages in the treatment of fatty oils. For example, it is possible to materially accelerate the rate of bodying of a fatty oil. It is further possible to materially improve the drying characteristics of the fatty oil, and also to improve water and alkali resistance of film coatings or the like formed with the treated oil. Still further, the treatment yields a modified oil which has special advantages in the field of electrical insulation, since the modified oil yields coatings having increased dielectric strength.

The foregoing and other objects and advantages will be considered more fully hereinafter following a description of two illustrative processes. However, before proceeding with the description, reference is now made to the fatty oil materials to which the invention is applicable.

## FATTY OIL

The process may be employed on fatty oils generally, including drying oils, semi-drying oils, and non-drying oils. The following is a typical list of such oils.

Tung oil  
Oiticica oil  
Dehydrated castor oil  
Linseed oil  
Perilla oil  
Sunflower oil  
Poppyseed oil  
Soya bean oil  
Walnut oil  
Rapeseed oil  
Pine seed oil

Olive oil  
Corn oil  
Cottonseed oil  
Coconut oil  
5 Babassu oil  
Hydroxylated oils such as castor oil, etc.  
Fish oils (train oils)

10 Synthetic esters of the fatty acids of the above mentioned oils behave similarly to fatty oils in the present process. Such synthetic esters may incorporate glycerine or other polyhydric alcohols, such as glycols, penta-erythritol, mannitol, sorbitol, etc.

15 The process may be employed on fatty oils themselves or on various mixtures of materials containing fatty oils, for instance on varnishes, in which event the fluorescein may conveniently be added at the time of cooking the varnish, so that the several ingredients of the varnish solids, are, so to speak, jointly treated or modified.

## FIRST ILLUSTRATIVE PROCESS

20 A batch of linseed oil is heated together with 2% of fluorescein, the temperature being maintained at about 300° C. for 5 hours. Vacuum is applied during the treatment period and the pressure maintained at about 100 mms. Hg.

The modified oil is a heavily bodied oil of an orange color, having a very strong fluorescence.

25 A varnish made with the treated oil has an unusually strong gel skeleton, which results in improved drying properties, especially in the initial drying stage, so that the varnish reaches the "print-free" stage very quickly. In addition the resistance to hot water and alkali of a varnish made with the treated oil is unusually good, cold water resistance also being at least equivalent to a varnish made with the same oil heated under the same conditions but without the fluorescein.

30 Varnish films made with the treated oil display a markedly improved dielectric strength.

## SECOND ILLUSTRATIVE PROCESS

35 Various of the foregoing improvements are also obtainable by employment of an alternative process wherein the fluorescein is made in situ, i. e., by treating the oil with resorcinol and phthalic anhydride added as such. In the case of this treatment, the resorcinol and phthalic anhydride are desirably added in those chemical proportions which are capable of combining to form the fluorescein. The molecular proportion of the two ingredients is two molecules of resorcinol for each 50 one molecule of phthalic anhydride. To achieve

this molecular proportion, the weight proportion should be about two parts of phthalic anhydride to three parts of resorcinol.

As the second illustrative process, therefore, a batch of linseed oil is treated with .2% of phthalic anhydride and .3% of resorcinol, the mixture being heated to about 300° C. under a pressure of 100 mms. Hg for a period of 5 hours.

Although the bodying rate is not increased to the same extent as when employing pre-condensed fluorescein, the oil treated with phthalic anhydride and resorcinol displays similarly improved drying properties and water and alkali resistance.

In addition, when forming the fluorescein in situ the color of the modified oil is very excellent for many purposes, being very light in color, and not displaying the distinctive orange shade characteristic of treatment with pre-condensed fluorescein.

Improved dielectric strength is also noted in varnish films made with oil treated with phthalic anhydride and resorcinol.

A number of variations may be introduced in either of the foregoing illustrative processes, these variations being mentioned more fully hereinafter following the specific examples which are given just below.

In considering the following examples, and in other discussion in the present specification, it is to be understood that statements regarding changes in properties and comparisons thereof are always made on the basis of a relation between the product treated with the modifying agent and a product treated in exactly the same manner (heating, etc.) but without a modifying agent. The latter is often herein referred to as a "blank" or "control" experiment.

Temperatures are always given in degrees centigrade, and viscosities are identified on the Gardner scale, unless otherwise specified. All parts mentioned are by weight.

#### EXAMPLES

Several comparative series of experiments were conducted in order to demonstrate the effect of varying the proportion of modifying agent. In one such comparative series, presented in Table I herebelow, a batch of 300 gms. of alkali refined linseed oil was heated in a 1 liter aluminum beaker, and a blanket of CO<sub>2</sub> gas maintained over the surface of the batch. In this series pre-condensed fluorescein was used and the batch of each experiment was heated for 5 hours at 300° C.

Varnishes were prepared from the treated oils of the several experiments, each varnish being a 25 gallon long varnish prepared as follows:

Two parts of the oil product and one part of an ester gum having a medium acid number were heated to 300° C. and kept at that temperature for 1 hour. The mixture was cooled to 200° C. and diluted with mineral spirits to 50% solids. Naphthenate driers were added in the proportion of .03% cobalt metal, .02% manganese metal and .30% lead metal, based on the quantity of oil used.

The varnishes were tested for drying, cold water resistance, hot water resistance, and alkali resistance.

A "blank" experiment on the same alkali refined linseed oil was also conducted under exactly the same treatment conditions (temperature, etc.) but without the fluorescein; and a varnish was prepared from this "blank."

The results of the several experiments of the series and of the "blank" are indicated in the following table:

Table I.—Fluorescein

| Ex. No. | The oil |           |                   | The varnish |               |           | Alkali resistance |
|---------|---------|-----------|-------------------|-------------|---------------|-----------|-------------------|
|         | Percent | Viscosity | Drying            | Cold water  | Boiling water |           |                   |
| A       | Blank   | Z4.....   | Fair.....         | Fair.....   | Fair.....     | Fair..... | Fair.             |
| 1       | .05     | Z2.....   | Superior.....     | Equal.....  | do.....       | do.....   | Equal.            |
| 2       | .5      | Z6.....   | do.....           | do.....     | do.....       | do.....   | Do.               |
| 3       | 2.0     | Gel.....  | do.....           | do.....     | do.....       | do.....   | Superior.         |
| 4       | 5.0     | do.....   | Far superior..... | do.....     | do.....       | do.....   | Far superior.     |

Designations in the "Varnish" columns express relation to the blank.

The testing of the varnishes was done in the following manner:

Varnish film were applied to steel panels by means of a coating knife yielding a film .003 of an inch thick. The drying of the varnishes on the panels was observed both with respect to initial drying (in the first 5 hours), and also after overnight drying. After the panels had been left for 48 hours to insure through-drying, the panels were tested for cold water resistance, boiling water resistance and alkali resistance.

The test for cold water resistance was conducted by immersing one-half of each panel in cold water for 24 hours, and then observing the appearance of the films.

The test for boiling water resistance was effected by immersing one-half of each panel in boiling water for 15 minutes, and then observing the appearance of the films, particularly for milkiness and softness, but also for the speed with which the milky films returned to their original appearance upon drying in the air.

The test for alkali resistance was effected by immersing one-half of each panel in 3% sodium hydroxide solution, and observing the time when the alkali completely attacked and dissolved the films.

A similar series of experiments was conducted in the same general manner, except that the batch undergoing treatment was heated in a 1 liter distilling flask at a pressure of 100 mms. Hg instead of employing a CO<sub>2</sub> blanket. The results of this series are indicated in Table II just below:

Table II.—Fluorescein

| Ex. No. | The oil |             |                   | The varnish |               |                   | Alkali resistance |
|---------|---------|-------------|-------------------|-------------|---------------|-------------------|-------------------|
|         | Percent | Viscosity   | Drying            | Cold water  | Boiling water |                   |                   |
| B       | Blank   | Z5.....     | Fair.....         | Fair.....   | Fair.....     | Fair.....         | Fair.             |
| 5       | .05     | Z.....      | Equal.....        | Equal.....  | do.....       | do.....           | Equal.            |
| 6       | .5      | Z4.....     | Superior.....     | do.....     | do.....       | Far superior..... | Superior.         |
| 7       | 2.0     | Z6.....     | Far superior..... | do.....     | do.....       | Far superior..... | Far superior.     |
| 8       | 5.0     | Nearly gel. | Far superior..... | do.....     | do.....       | Equal.....        | Do.               |

#### Example 9

A batch of 300 gms. of dehydrated castor oil was heated, together with .05% fluorescein, in a 70 distilling flask, the temperature being maintained at about 300° C. for a period of one and one-half hours. The oil was of quite light color and reached a viscosity of Z6. A 25 gallon long varnish was prepared in the manner described above and when diluted to 50% solids reached a viscos-

ity of G. The varnish had good drying properties and good resistance to both hot and cold water, and in addition the varnish displayed excellent alkali resistance, the film still being intact after 24 hours immersion in the 3% sodium hydroxide solution.

*Example 10*

A similar experiment was conducted with dehydrated castor oil, employing 5% fluorescein. With this percentage, the mixture was heated for 46 minutes at 300° C., at the end of which time the viscosity was Z6<sup>++</sup>. The color of the oil was somewhat darker than that of Example 9.

A similar varnish was prepared in the manner outlined above, employing the oil of Example 10 and this varnish displayed good drying properties, as well as hot and cold water and alkali resistance.

Dehydrated castor oil with fluorescein shows very rapid bodying, if heavy bodied oils are being made. If a varnish is cooked out of such oils, the varnish bodying speed is also accelerated.

*Example 11*

A batch of 300 gms. of alkali refined linseed oil was heated in an open 1 liter aluminum beaker together with .5% fluorescein for 5 hours between about 295° C. and 305° C. A similar batch of oil without the fluorescein was treated in the same manner, as a "blank" experiment. The following tabulation indicates the comparative results secured with the "blank" (C) and with the fluorescein treated oil. The varnish was prepared in the same manner as that described above.

Table III.—Fluorescein

| Ex. No. | The oil |           | The varnish      |                  |                   |           |                       |                      |                   |
|---------|---------|-----------|------------------|------------------|-------------------|-----------|-----------------------|----------------------|-------------------|
|         | Color   | Viscosity | Color of varnish | Visc. of varnish | Drying properties |           | Cold water resistance | Hot water resistance | Alkali resistance |
|         |         |           |                  |                  | Initial           | Overnight |                       |                      |                   |
| 11----- | 13      | Z-3       | 15               | A                | VG                | VG        | VG                    | VG                   | Overnight.        |
| C-----  | 10      | Z-2       | 12               | A-               | F                 | F         | F                     | B                    | 5½ hours.         |

Key to chart:

Colors in Hellige comparator scale—

VG—very good.

F—fair.

B—bad.

*Example 12*

A batch of linseed oil was heated in a distilling flask with 5% of fluorescein under a pressure of about 50 mms. Hg. During initial heating there was a sudden rise in temperature from about 80° C. to about 160° C., accompanied by frothing, which, however, subsided at about 200° C. when some gas evolution occurred. Fifty minutes was required to reach 300° C. and after about one hour at 300° C., the batch had already thickened, and upon continuing the heating for a total of four hours the batch was almost solid. Further heating indicated a tendency for the oil to become somewhat more fluid.

The product was a thick sticky oil of golden brown color with green fluorescence.

*Example 13*

A batch of linseed oil (pre-dried of moisture content) was heated in an open iron beaker with 5% of fluorescein. About one and three-quarter hours was required to reach 290° C. The mixture was then kept between about 290° C. and 302° C. for one and three-quarter hours, and then permitted to cool overnight.

On starting the next day, the oil was noticed to be quite thick, but it quickly thinned on reheating, requiring about three-quarters of an hour to again reach 290° C. The batch was then kept between about 290° C. and 302° C. for an additional three and one-quarter hours, so that the entire time on temperature totaled five hours.

The product, when cooled, was a brown elastic jelly, with a strong green fluorescence.

10 25 gallon long varnishes were made with the oils of Examples 12 and 13 and in addition similar varnishes were made with the same oils treated in the same manner except for the omission of the modifying agent. The varnishes were made with lime hardened rosin. The varnishes were initially tested without driers, and both of the varnishes made with fluorescein-treated oils reached the final drying stage much more quickly than the two corresponding "blank" 15 varnishes. Upon addition of cobalt drier to the varnishes, the varnish made with the product of Example 13 dried much faster than the corresponding "blank" varnish.

20 Certain examples are also given below illustrating the use of fluorescein as applied to mixed materials, incorporating a fatty oil. Specifically, Examples 14, 15 and 16 illustrate the treatment of electrical insulating varnishes with fluorescein.

*Examples 14 and 15*

25 In each of Examples 14 and 15 an insulating varnish was prepared in the following manner, Example 14 employing 5% of fluorescein and Example 15, 2% of fluorescein (based on the oil content).

30

In each of Examples 14 and 15 an insulating varnish was prepared in the following manner, Example 14 employing 5% of fluorescein and Example 15, 2% of fluorescein (based on the oil content).

55 In each example 169 parts of alkali refined linseed oil and 20 parts of a modified phenolic resin (rosin modified) were initially heated to 300° C. together with the fluorescein and held at that temperature for two and three-quarter hours. 30 parts of lime hardened rosin were then added and the mixture reheated to 300° C. and held there for ten minutes. 10 parts of zinc resinate were added. Following the zinc resinate addition the batch was again reheated to 300° C. and held for one-half hour. Then driers were also added: 1.2 parts lead naphthenate drier (40% metallic lead content); and 1 part manganese naphthenate drier (10.5% metallic manganese content).

60 65 Finally the batch was permitted to cool to 220° C. and was cut with 215 parts mineral spirits, yielding approximately 50% solids. This varnish formula yields about a 35 gallon long varnish.

70 Various properties of the foregoing varnishes (Example 14 containing 5% fluorescein, and Example 15 containing 2% fluorescein) are indicated in the table below (Table IV). The table also includes a varnish representing a "blank" 75 experiment marked "D," this varnish being pre-

pared in essentially the same manner as that described above except for omission of the fluorescein.

Table IV.—Fluorescein

| Ex. No. | Specific gravity | Visc. | Drying time (hrs.) at 110° C. | Dielectric strength, dry | Volts per mil, wet | Heat endurance (life) in hours | Oil resistance hardness |
|---------|------------------|-------|-------------------------------|--------------------------|--------------------|--------------------------------|-------------------------|
| 14..... | 0.888            | I-J   | 2½                            | 1,585                    | 405                | 408                            | 378                     |
| 15..... | .886             | F     | 2                             | 1,820                    | 640                | 408                            | 250                     |
| D.....  | .884             | F-G   | 1½                            | 1,385                    | 330                | 312                            | 300                     |

All of the tests indicated in the above table were made in accordance with A. S. T. M. methods. In addition it may be noted that while the "blank" had a rating (A. S. T. M.) of 51, the varnish of Example 14 had a rating of 52 and that of Example 15 had a rating of 60.

## Example 16

Another insulating varnish was prepared in a manner similar to that described above, with the following differences:

The lime hardened rosin and the zinc resinate were replaced by ester gum, the other ingredients remaining unchanged and the procedure in heating, etc., being essentially the same. In this case the total cooking time was three hours and 5% of the fluorescein was used. A "blank" experiment was also conducted (with a total cooking time of three and one-half hours) and the comparison of Example 16 with the "blank," marked "E," is given just below:

Table V.—Fluorescein

| Ex. No. | Specific gravity | Visc. | Drying time (hrs.) at 110° C. | Dielectric strength, dry | Volts per mil, wet | Heat endurance (life) in hours | Oil resistance hardness |
|---------|------------------|-------|-------------------------------|--------------------------|--------------------|--------------------------------|-------------------------|
| 16..... | 0.890            | R     | ¾                             | 1,870                    | 775                | Over 1,000                     | 500                     |
| E.....  | .882             | A—    | ¾                             | 1,770                    | 545                | Over 1,000                     | 375                     |

<sup>1</sup> Tack.

The varnish of Example 16 indicated a rating of 80+, which compared with 60+ for the "blank" "E." Note the high viscosity of the varnish 16 with fluorescein and the extremely low viscosity of the corresponding "blank" "E."

The foregoing tables indicate that employment of fluorescein in insulating varnishes increases to a great extent the dielectric strength, both when wet and when dry, the varnishes employing fluorescein also yielding quite rapid baking time, long life and fair oil resistance. Comparison of the two sets of experiments (on insulating varnishes) further show that substitution of ester gum for the lime hardened rosin and zinc resinate further improve the qualities of the varnish.

In order to demonstrate the effect of treating a fatty oil with phthalic anhydride and resorcinol, so as to form the fluorescein in situ, some additional comparative experiments were conducted, these being treated of under Examples 17 and 18 below. In all experiments of these two series the phthalic anhydride and resorcinol were used in relative proportions of 2 to 3 by weight. In the discussion just below it is to be understood that the percentage of reagent given indicates the total percentage of the two ingredients in the proportions just mentioned.

## Example 17

Batches of 5,000 gms. of alkali refined linseed oil were heated in aluminum pots under CO<sub>2</sub>

blanket, the temperature being 300° C. The following percentages were used, some with, and some without mechanical agitation, as indicated. All batches were heated until the oil reached a body of from Z5 to Z6.

- (a) .05% of the reagent mixture was used with agitation.
- (b) .05% of the reagent mixture was used without agitation.
- (c) .1% was used without agitation.
- (d) .5% was used without agitation.
- (e) 2% was used with agitation.
- (f) 5% was used with agitation.
- (g) A "blank" experiment was also conducted without agitation.

## Example 18

A similar group of experiments was conducted on batches of 8,000 gms. of alkali refined linseed oil heated in a 22-liter distilling flask under vac-

uum (pressure 100 mms. Hg). Here again the temperature was 300° C. and the oils were heated until a body of Z5 to Z6 was attained.

- (a) .5% was used with agitation.
- (b) .5% was used without agitation.
- (c) A "blank" experiment was conducted without agitation.

Although the rate of bodying of the oil in general, was only slightly accelerated in the two examples just above noted, it is of importance to note that the oil products were consistently of very light color.

The oils of Examples 17 and 18 were used in making up 25 gallon long ester gum varnishes which were cooked to C-H viscosity at 50% solids in mineral spirits, the varnishes thereafter being tested for drying properties, cold water resistance, boiling water resistance, and alkali resistance.

With respect to the preparation of the varnishes with the above oils it is of importance to note that the time required to cook the varnish to a given body (varnish bodying time) was materially decreased by the employment of the oils treated with phthalic anhydride and resorcinol. Especially fast bodying of the varnish was shown in the varnishes made up as indicated under (a) and (d) of Example 17 and (a) of

Example 18. Improvement in varnish bodying time was as much as 20 to 30%.

With respect to drying of these varnishes, it may be noted that they indicated somewhat faster initial drying, and in many cases very definitely improved through drying in an overnight period. This is especially true of items (a), (b), (e) and (f) of Example 17 and also of items (a) and (b) of Example 18.

Cold and boiling water resistance tests indicated results at least equivalent to the "blank" experiments. The alkali resistance of the varnishes prepared with the oils treated with the reagent mixture was consistently better than the "blank," although the improvement in this respect is not as notable as where the fluorescein is used in pre-condensed form.

#### RANGES AND VARIATIONS OF TREATMENT

In addition to the examples given above, it has been demonstrated by other actual examples that effective results are secured by first preparing a master batch of a fatty oil containing a relatively high percentage of phthalic anhydride and resorcinol, and thereafter diluting a relatively large batch of fatty oil with the master batch. This has the advantage of enabling the preparation of relatively large quantities of oil in relatively small equipment, since only the master batch need be specially handled. In one instance master batches containing 20% of phthalic anhydride and resorcinol (in the relative proportions of 2 to 3) were prepared by heating only until the modifying agents are completely dissolved in the oil, these master batches being used thereafter to dilute larger quantities of oil so as to yield oil products containing various percentages of the combined reagent, for instance as above referred to in Examples 17 and 18. The properties of the oils prepared in this way were similar to those prepared in accordance with the methods of Examples 17 and 18.

In connection with the modifying agent it may be mentioned that substituted fluorescein, its derivatives and salts may also be used. Moreover, in the alternative process (preparation of the modifying agent *in situ*) materials may be used which yield either fluorescein itself, or substituted fluorescein, its derivatives and salts.

With respect to variations of temperature, etc., 50 note the following:

The temperature in treating an oil with fluorescein may be anywhere from about 200° C. up to about 350° C., preferably not above the point at which the oil boils or decomposes. An effective range has been found to be from about 250° C. to about 310° C.

When using phthalic anhydride-resorcinol mixtures, a master batch may be mixed into oils even cold, and such oils may react with the agents either while bodying oils and/or while cooking varnishes with such oils.

Although under at least some circumstances, the modifying agent may be employed in a relatively high percentage, for instance up to about 30%, when using fluorescein the quantity should not usually be above about 10%, especially because of the fact that the fluorescein is difficultly soluble in fatty oils. An effective range for fluorescein is from about .05% to about 5%. However, in the event of using certain auxiliary agents or resins (such as are used in varnish cooking), dissolution of the fluorescein may be promoted, in which event more than 10% may be employed.

When using phthalic anhydride-resorcinol mixtures the reagent may be employed up to 20% or even 30%, although an effective range is from about .05% to about 10%.

5 The time will vary depending upon the other conditions of the process, such as percentage, temperature, etc., and also upon whether or not the fluorescein is employed in pre-condensed form or is formed *in situ*. Note for instance that to achieve a given body when treating an oil, greater time is required when forming the fluorescein *in situ* than when employing pre-condensed fluorescein. In the latter case, in fact, extremely rapid bodying is obtainable. As a general guide it may be said that a few hours, for instance from about 1 hour to about 5 or 10 hours is sufficient. With certain oils, and under certain conditions (note for instance Examples 9 and 10, above, using dehydrated castor oil), extensive bodying takes place even in a matter of minutes.

20 The treatment may be carried out under varying atmospheric conditions, both with respect to pressure and also with respect to the gas in contact with the reaction mixture. Thus, in examples given above, certain oils were treated under vacuum and others at atmospheric pressure. Moreover, some of the examples employed a blanket of CO<sub>2</sub>.

30 It is frequently of advantage to exclude the air from a reaction mixture and this may be done either by employing vacuum or by blanketing the surface of the batch with some inert gas, for instance, CO<sub>2</sub>, SO<sub>2</sub>, H<sub>2</sub>S, or nitrogen. Still further exclusion of air may be obtained by carrying out the reaction in a closed vessel (but not necessarily under a positive pressure), in which event vapors or the like released from the reaction mass may serve to dispel or exclude the air. I have 40 found vacuum treatment to be particularly effective, for instance from about 100 mms. Hg to about 450 mms. Hg, although higher or lower pressures are also useable.

45 With regard to the foregoing atmospheric conditions in the reaction vessel, it may be noted that certain of the gases mentioned may be employed for their supplemental effect on the reaction, in which event, if desired, the gases may be bubbled through the reaction mixture.

In general it may be pointed out that increasing any one of the temperature, time or percentage of modifying agent usually increases the rate and/or extent of the reaction.

55 The modifying agent herein claimed may be employed (either simultaneously or sequentially) in combination with others disclosed, for instance, in various of my copending applications and issued patents, some of which are mentioned hereinafter. Interesting results may be obtained for instance when oils made according to my copending application 383,339 now Patent No. 2,298,915 are after-treated according to the present process. Examples of such other modifying agents are anthraquinone derivatives.

60 65 In addition, supplemental treatments may be applied to the oil, either during or following the reaction with fluorescein, many of such supplemental treatments also being discussed fully in copending applications and issued patents below mentioned. For instance, the modified oil products may be vulcanized with sulphur or sulphur chloride or similar vulcanizing agents.

70 75 Particularly effective results are secured with a vulcanized oil product, where the oil has been treated with fluorescein or with phthalic anhy-

dride and resorcinol. It is found that when such products are compounded with rubber, they display appreciably improved characteristics from the standpoint of tensile strength.

As hereinabove mentioned the present application is a continuation-in-part of my copending application Serial No. 383,339 now Patent No. 2,298,915 issued October 13, 1942. Certain subject matter disclosed herein is also disclosed in my copending application Serial No. 318,650 filed February 12, 1940 now Patent No. 2,298,270 issued October 13, 1942, and also in application Serial No. 359,425 (now patent No. 2,213,944). Application 446,170 (now Patent 2,234,949), of which Serial No. 318,650 is a continuation-in-part, also presents similar subject matter.

I claim:

1. The method of modifying a fatty oil to improve its drying characteristics which comprises incorporating in the oil up to 30% of fluorescein and heating the mixture to a temperature between about 200° C. and about 350° C. but not above the boiling point of the oil.

2. The method of modifying a fatty oil to improve its drying characteristics which comprises incorporating in the oil up to 10% of fluorescein, and heating the mixture to a temperature between about 200° C. and 350° C. but not above the boiling point of the oil.

3. A process in accordance with claim 2 in which the fluorescein is present in an amount from about .05% to about 5%.

4. The method of modifying a fatty oil to improve its drying characteristics which comprises incorporating in the oil up to 30% of a modifying agent comprising phthalic anhydride and resorcinol, and heating the mixture to a temperature between about 200° C. and 350° C. but not above the boiling point of the oil, the phthalic anhydride and resorcinol being employed in proportions in which they combine chemically with each other.

5. A process in accordance with claim 1 in which the quantity of the fluorescein is from about .05% to about 10%.

6. A process in accordance with claim 1 in which the fatty oil is linseed oil.

7. A process in accordance with claim 1 in which the fatty oil is soya bean oil.

8. A process in accordance with claim 1 in which the fatty oil is a castor oil.

9. A process in accordance with claim 1 in which the fatty oil is dehydrated castor oil.

10. A process in accordance with claim 1 in which the fatty oil is treated in admixture with a varnish resin comprising rosin.

11. In the preparation of varnishes, the process which comprises cooking a resin-plus-oil mixture together with up to 20% of fluorescein, the cooking being effected at oil bodying temperature.

12. A process in accordance with claim 11 in which the fluorescein is employed in an amount from about .05% to about 5%.

13. A process for treating fatty oils which comprises first dispersing a relatively high percentage of a modifying agent comprising phthalic

anhydride and resorcinol in a master batch of fatty oil, and thereafter combining oil of said master batch with a larger quantity of fatty oil, and heating the resulting mixture to heat bodying temperatures, the phthalic anhydride and resorcinol being employed in proportions in which they combine chemically with each other.

14. A heat bodied fatty oil product having dispersed therein the reaction product of up to 10% of fluorescein with the fatty oil, the quantity of the reacted fluorescein being based on the heat bodied fatty oil product.

15. The method of modifying a fatty oil which comprises dispersing in the oil up to 30% of a modifying agent comprising phthalic anhydride and resorcinol, heating the oil, subsequent to dispersion of the modifying agent, to a temperature between about 200° C. and 350° C., the phthalic anhydride and resorcinol being employed in proportions in which they combine chemically with each other.

16. The process of claim 1, in which the modified fatty oil is heated with sulfur to form a vulcanized fatty oil product.

17. A heat bodied fatty oil material comprising the reaction product of fluorescein formed with the fatty oil, the quantity of the reacted fluorescein being up to 30% of the heat bodied fatty oil material.

18. A vulcanized heat bodied fatty oil material comprising the reaction product of fluorescein formed with the fatty oil, the quantity of the reacted fluorescein being up to 30% of the heat bodied fatty oil material.

19. A heat bodied fatty oil material comprising the reaction product of phthalic anhydride and resorcinol formed with the fatty oil, the quantity of the reacted phthalic anhydride and resorcinol being up to 30% of the heat bodied fatty oil material.

20. A vulcanized heat bodied fatty oil material comprising the reaction product of phthalic anhydride and resorcinol formed with the fatty oil, the quantity of the reacted phthalic anhydride and resorcinol being up to 30% of the heat bodied fatty oil material.

21. The process in accordance with claim 1 in which the fluorescein is formed in situ under the conditions of the treatment from phthalic anhydride in admixture with resorcinol.

22. A heat bodied fatty oil material comprising the reaction product of phthalic anhydride and resorcinol formed with the fatty oil, the quantity of the reacted phthalic anhydride and resorcinol together being up to 30% of the heat bodied fatty oil material and the proportion of phthalic anhydride to resorcinol being approximately one mol to two mols.

23. A process in accordance with claim 11, in which the fluorescein is formed in situ under the conditions of the treatment from phthalic anhydride in admixture with resorcinol, the sum of the quantity of phthalic anhydride and resorcinol employed being from about 0.05% to about 10%.

LASZLO AUER.